

[54] RUBBING SEAL FOR A ROTARY  
REGENERATIVE HEAT EXCHANGER[75] Inventors: **Calvin Eric Silverstone; Alan John Surrall**, both of Solihull, England[73] Assignee: **Leyland Gas Turbines Limited**, Solihull, England[22] Filed: **June 1, 1971**[21] Appl. No.: **148,529**

## [30] Foreign Application Priority Data

June 26, 1970 Great Britain.....31,069/70

[52] U.S. Cl. .... **277/96 R**, 106/63, 165/9,  
277/DIG. 6[51] Int. Cl. .... **F16j 15/16**[58] Field of Search.....165/9; 277/96 R,  
277/DIG. 6; 106/39 R, 55, 63

## [56]

## References Cited

## UNITED STATES PATENTS

|           |         |                       |         |
|-----------|---------|-----------------------|---------|
| 3,646,993 | 3/1972  | Rice et al. ....      | 165/9   |
| 3,204,969 | 9/1965  | Williams.....         | 165/9 X |
| 3,351,127 | 11/1967 | Mendelsohn.....       | 165/9   |
| 3,633,926 | 1/1972  | Hryniszak et al. .... | 165/9 X |

Primary Examiner—Albert W. Davis, Jr.  
Attorney—Mawhinney & Mawhinney

## [57]

## ABSTRACT

A rubbing seal for engagement with a hot face of a matrix of a rotary regenerative heat exchanger. The seal comprises a ferritic steel base member, a rubbing surface layer including nickel oxide and an intermediate bonding layer of a nickel aluminum compound between the base member and the rubbing surface layer.

2 Claims, 1 Drawing Figure



PATENTED MAY 1 1973

3,730,538



INVENTORS  
CALVIN ERIC SILVERSTONE,  
ALAN JOHN SURRELL

## RUBBING SEAL FOR A ROTARY REGENERATIVE HEAT EXCHANGER

The invention relates to a rubbing seal for a rotary regenerative heat exchanger and is particularly concerned with a rubbing seal for engagement with a hot face of the matrix of a rotary regenerative heat exchanger for a gas turbine engine.

Existing rubbing seals for engagement with a hot face of the matrix of a rotary regenerative heat exchanger have been formed by depositing a layer containing nickel oxide and calcium fluoride on to an austenitic stainless steel base member. Such a seal has suffered from the disadvantage that at high engine operating temperatures, the deposited layer has become detached from the base member. The reason for this is believed to be that there is a difference between the expansion co-efficient of stainless steel and that of nickel oxide, the approximate expansion co-efficient of stainless steel being  $18 \times 10^{-6}/^{\circ}\text{C}$  and that of nickel oxide being  $13 \times 10^{-6}/^{\circ}\text{C}$ . An object of this invention is to provide a rubbing seal in which the co-efficients of expansion of the material of the base member and of the actual seal material are substantially the same.

Another disadvantage of the existing seal is that the seal material contains calcium fluoride, thereby giving rise to a health hazard. Therefore another object of the invention is to avoid the use of calcium fluoride in the rubbing seal material.

According to the invention a rubbing seal, for engagement with a hot face of a matrix of a rotary regenerative heat exchanger, comprises a ferritic steel base member and a rubbing surface layer including nickel oxide.

The seal may include an intermediate bonding layer of a nickel aluminum compound. A suitable material is available commercially as Metco 405, a material manufactured by Metco Limited.

The rubbing surface layer may be formed from a powder comprising a mixture of nickel oxide and calcium carbonate, the quantity of the latter by weight being not more than 10 percent of the total composition of the powder. Alternatively the powder may comprise a mixture of nickel oxide, metallic nickel and calcium carbonate, the quantity of nickel and calcium carbonate by weight being not more than 25 percent and 10 percent respectively of the total composition of the powder.

By way of example, a rubbing seal in accordance with the invention comprises a base member of a ferritic steel, instead of using an austenitic stainless steel as hitherto. The ferritic steel base member maybe protected against oxidation by depositing on it a bonding layer of a nickel aluminum compound, for example, that known as Metco 405. The deposition of the com-

5 pound is conveniently effected by a flame gun. A rubbing seal layer is formed on the bonding layer or, where a bonding layer is not required, directly on to the ferritic steel base member, by depositing with a flame gun a powder containing nickel oxide. The powder employed may either be a mixture of nickel oxide and calcium carbonate, the quantity of the latter by weight being not more than 10 percent or a mixture of nickel oxide, metallic nickel and calcium carbonate, the quantities of nickel and calcium carbonate by weight being not more than 25 percent and 10 percent respectively.

10 A section through a typical rubbing seal in accordance with the foregoing example is illustrated in the accompanying drawing. The seal comprises a ferritic steel base member 1 attached, by welding, brazing or otherwise, to a metal bellows 2. The bonding layer of the nickel aluminum compound, e.g., Metco 405, is shown at 3. This, as aforesaid, is conveniently deposited on the base member by using a flame gun. The actual rubbing seal material which is deposited on to the bonding layer 3 by flame deposition is shown at 4.

15 The wear rate of the layer formed by flame deposition of nickel oxide and calcium carbonate is similar to that produced from a nickel oxide and calcium fluoride mix, but the wear rate of the alternative mixture of nickel oxide, metallic nickel and calcium carbonate has approximately ten times less wear rate than the known rubbing seal composition using nickel oxide and calcium fluoride. It is believed that the reason for this significant improvement in wear rate lies in the higher density of the deposit resulting from the in situ oxidation of the nickel in the powder mixture.

20 In either case the powder mixture has an expansion co-efficient similar to that of the ferritic steel base of approximately  $13 \times 10^{-6}/^{\circ}\text{C}$ .

25 The powder mixtures proposed herein are cheaper to produce than mixtures used at present as they do not include calcium fluoride and furthermore the health hazard arising from calcium fluoride is not present.

30 What we claim as our invention and desire to secure by Letters Patent of the United States is:

35 1. A rubbing seal for engagement with a hot face of a matrix of a rotary regenerative heat exchanger, the seal comprising a ferritic steel base member and a rubbing surface layer formed from a powder comprising a mixture of nickel oxide, metallic nickel and calcium carbonate, the maximum quantity of nickel and calcium carbonate by weight being 25 percent and 10 percent respectively of the total composition of the powder.

40 2. A seal as claimed in claim 1 in which there is an intermediate bonding layer of a nickel aluminum compound between the base member and the rubbing surface layer.

\* \* \* \* \*